

# United States Patent

[19]

Kennedy

[11] 3,912,826

[45] Oct. 14, 1975

[54] **METHOD OF PHYSICAL VAPOR  
DEPOSITION**

3,504,325 3/1970 Rairden ..... 117/93.3  
3,751,310 8/1973 Cho ..... 117/93.3

[75] Inventor: **Kurt D. Kennedy, Berkeley, Calif.**

*Primary Examiner*—John H. Newsome  
*Attorney, Agent, or Firm*—Fitch, Even, Tabin &  
Luedeka

[73] Assignee: **Airco, Inc., Montvale, N.J.**

[22] Filed: **Jan. 14, 1974**

[21] Appl. No.: **432,874**

**Related U.S. Application Data**

[63] Continuation-in-part of Ser. No. 282,388, Aug. 21,  
1972, abandoned.

[52] **U.S. Cl.** ..... 427/8; 427/13; 427/38

[51] **Int. Cl.<sup>2</sup>** ..... C23C 13/02; C23C 13/04

[58] **Field of Search** ..... 117/93.3, 93.1 GD, 93.4 R,  
117/106 R

[56] **References Cited**

**UNITED STATES PATENTS**

3,290,567 12/1966 Gowen ..... 117/93.3

[57]

## **ABSTRACT**

A method of physical vapor deposition is described wherein a source of evaporant material and a substrate are placed in a vacuum chamber maintained at a pressure of less than  $10^{-4}$  Torr. A vapor of the evaporant material is produced for deposition on the substrate. The vapor is intercepted with the beam of electrons to produce positive ions, and the substrate is maintained at a negative electrical potential sufficient to cause substantial heating of the substrate by ion bombardment.

**4 Claims, No Drawings**

## METHOD OF PHYSICAL VAPOR DEPOSITION

This application is a continuation-in-part of application Ser. No. 282,388 filed Aug. 21, 1972, now abandoned.

This invention relates to physical vapor deposition and, more particularly, to an improved method for physical vapor deposition under conditions of elevated substrate temperatures.

Physical vapor deposition of materials on substrates is of considerable advantage in many production operations. Physical vapor deposition is generally carried out in a relatively high vacuum environment in which the material to be deposited is evaporated by raising it to a sufficiently high temperature. The required heat may be produced by suitable heating, such as by electron beams.

For some types of materials, it is desirable to elevate the substrate temperature and maintain it at the elevated temperature during the physical vapor deposition process. In some cases, this is done to enhance ductility in the resulting deposit. In other cases, it is done to enhance the adhesion between the deposit and the substrate, or to achieve a desired crystalline configuration in the deposit. Typically, the substrate is heated to a temperature which is at least 25% of its absolute melting temperature, and often, the heating is to substantially higher temperatures.

During the coating operation, a certain amount of heat input will occur into the substrate as a result of the latent heat of vaporization in the condensing vapor. At temperatures up to about 500°F, the heat input from the coating itself, as a result of the latent heat of vaporization, is usually sufficient to maintain a desired temperature. Above about 500°F, however, it is typically necessary to provide an additional source of heat for the substrate during the coating process.

One means of heating substrates being coated is shown and described in U.S. Pat. No. 3,560,252, assigned to the assignee of the present invention. The technique described in the aforesaid patent has proved to be of substantial and significant commercial importance. Certain types of substrates, however, do not readily lend themselves to heating by radiant heaters. For example, strip lines in which a continuous strip of substrate is fed into and out of a vacuum chamber may render radiant heating somewhat inconvenient.

Accordingly, it is an object of the present invention to provide an alternative means of substrate heating to the use of radiant heaters.

Another object of the invention is to provide an improved method of physical vapor deposition.

It is another object of the invention to provide an improved method of physical vapor deposition which is particularly suited to continuous strip substrates.

Other objects of the invention will become apparent to those skilled in the art from the following description.

Very generally, the method of the invention is directed to depositing an evaporant material on a substrate. A source of evaporant material and a substrate are placed in a vacuum chamber. The vacuum chamber is maintained at an ambient pressure of less than  $10^{-4}$  Torr. A vapor of the evaporant material is produced in the vacuum chamber for deposition on the substrate. A beam of electrons is directed at the vapor to produce positive ions. An electrical potential is maintained on

the substrate which is sufficient to cause substantial heating of the substrate by ion bombardment.

Referring now to the invention in greater detail, the method of the invention is practiced, preferably, in an electron beam furnace or similar apparatus. Apparatus of this general type is illustrated schematically in the previously mentioned U.S. patent. Also, apparatus of this general type is well known to those skilled in the art, and therefore will not be described in detail herein.

10 Typically, the electron beam furnace used for physical vapor deposition comprises an evacuated enclosure, means for maintaining a pressure in the enclosure (other than in the vapor cloud), hereinafter referred to as the ambient pressure, of less than  $10^{-4}$  Torr. A vapor 15 of the evaporant material is produced from a molten pool or by sublimation from a solid, by suitable heating. Preferably, this is accomplished by means of an electron beam directed at a solid or liquid source of the evaporant. After the vapor cloud is produced, the 20 cloud is allowed to intercept the substrate such that evaporant condenses on the surface of the substrate, providing the coating.

In order to produce the vapor, the target evaporant material is heated by any suitable means. Preferably, such heating is accomplished by an electron beam directed on to the surface of the evaporant material by suitable magnetic fields.

Typically, a substantial portion of the vapor cloud thus produced is intercepted by the electron beam. The 25 impingement of electrons upon the vapor particles produces ionization and, consequently, a large number of positive ions are present in the chamber.

Typically, a substantial portion of the vapor cloud thus produced is intercepted by the electron beam. The 30 impingement of electrons upon the vapor particles produces ionization and, consequently, a large number of positive ions are present in the chamber.

As will be explained, the positive ions thus produced are utilized, in accordance with the invention, to produce heating of the substrate. To this end, the substrate is maintained at an electrical potential sufficient to cause substantial heating of the substrate by ion bombardment. This is accomplished by adjusting the operating pressure in the system, such as by bleeding in a 35 suitable inert gas such as Argon, and by adjusting the bias potential on the substrate, such that the heat input balances the heat output at the desired substrate temperature, thus establishing a condition of equilibrium.

The heat output, of course, is principally through the 40 mode of radiation, especially in the case of discrete substrates. Some conduction, however, will occur. For example, in the case of discrete substrates, conduction will occur through the mechanical means by which the discrete substrate is supported. Even greater heat loss 45 through conduction will occur in the case of a moving strip, since heat is conducted along the strip both in the upstream and downstream directions. Thus, it is typically more expedient to establish the equilibrium conditions empirically through experimental set-ups, rather than attempting to calculate them in advance.

The potential may be either a high negative potential with respect to the source, or may be a high alternating current potential. In either case, the potential is preferably great enough to accelerate a sufficient number of

50 positive ions to the substrate so as to provide a power density on the substrate of about 6 or  $6\frac{1}{2}$  watts per square inch of exposed surface. The vapor source will, of course, supply some radiant heat and therefore the larger and hotter the vapor source is, the less ion heating 55 that is required to achieve a given temperature.

The amount of potential required for accelerating sufficient ions depends upon the amount of ions available. This, of course, depends upon the pressure in the

system including the amount of vapor present (i.e. the evaporation rate). Thus, in cases where material such as zinc is being evaporated, typically providing very

input was below the desirable minimum level and therefore provided a substrate temperature of only 340°F.

| Ex.No. | Pressure<br>(micron) | Bias Volt.<br>(KV) | Current<br>(amps.) | Pwr. Input<br>(watts/sq. in) | Subst. Temp.<br>°F |
|--------|----------------------|--------------------|--------------------|------------------------------|--------------------|
| 11     | 50                   | 1.0                | 0.02               | 5                            | 340                |
| 12     | 50                   | 1.5                | 0.04               | 15                           | 600                |
| 13     | 50                   | 2.0                | 0.06               | 30                           | 700                |
| 14     | 50                   | 2.5                | 0.08               | 50                           | 850                |
| 15     | 50                   | 3.0                | 0.10               | 75                           | 920                |
| 16     | 50                   | 3.5                | 0.12               | 105                          | 1600               |

high evaporation rates, only 1 KV or less bias voltage will be required for the requisite heating. On the other hand, where a relatively low evaporation rate exists, bias voltages of 10 KV or greater may be required. Some lessening of the required voltage may be obtained by raising the system pressure through use of an inert gas bleed.

The following Table illustrates the effect of changes in pressure on current and hence power input to the substrate in a deposition set-up. Examples 1-5 relate to the heating of a stainless steel disc 11 inches in diameter providing a surface area of about 190 sq. inches. The second group of examples, 6-10, relates to the coating of a 2 inch square stainless steel substrate 0.080 inches thick, thus providing a surface area of 4 square inches. In each case, the pressure of the system in microns is given, the bias voltage on the substrate (held steady) in kilovolts is given, the measurable electrical current flowing into the substrate as a result of ion bombardment is given, the approximate temperature of the substrate at equilibrium is given, and the input power density to the substrate in watts per square inch is also given.

15 For precise control of substrate heating, it may be desirable to provide a closed loop arrangement. Thus, suitable sensors may be employed to sense the temperature of the substrate and provide an electrical signal related thereto. This electrical signal may then be utilized to regulate or control the bias voltage on the substrate, thereby maintaining a relatively constant substrate temperature. The circuitry required for such an electrical arrangement will be readily apparent to those skilled in the art.

20 25 It may therefore be seen that the invention provides an improved method of physical vapor deposition in which substrate heating is accomplished by the acceleration of ions present in the vapor cloud to impinge upon the substrate. The invention is particularly suitable for situations in which substrate heating by other means, such as by radiant heaters, is undesirable or impractical.

30 35 Various modifications of the invention in addition to those shown and described herein will become apparent to those skilled in the art from the foregoing description. Such modifications are intended to fall within the scope of the appended claims.

| Ex. No. | Pressure<br>(micron) | Bias Volt.<br>(KV) | Current<br>(amps.) | Pwr. Input<br>(watts/sq.in.) | Subst. Temp.<br>°F |
|---------|----------------------|--------------------|--------------------|------------------------------|--------------------|
| 1       | 50                   | 3.5                | 0.8                | 20                           | 650                |
| 2       | 40                   | 3.5                | 0.76               | 14                           | 580                |
| 3       | 30                   | 3.5                | 0.52               | 9.6                          | 550                |
| 4       | 20                   | 3.5                | 0.36               | 6.6                          | 500                |
| 5       | 10                   | 3.5                | 0.03               | 5.5                          | 300                |
| 6       | 50                   | 3.5                | 0.04               | 35                           | 1600               |
| 7       | 40                   | 3.5                | 0.04               | 35                           | 950                |
| 8       | 30                   | 3.5                | 0.06               | 52.5                         | 850                |
| 9       | 20                   | 3.5                | 0.08               | 70                           | 700                |
| 10      | 10                   | 3.5                | 0.12               | 105                          | 500                |

As may be seen from the Table, example 5 resulted in an equilibrium temperature below that which is commercially significant, since such a low equilibrium temperature could be achieved by suitable adjustments in the evaporation rate and without a substrate bias. It may also be seen that a power input density of at least about 6 or 6½ watts per square inch is typically necessary to achieve the desired minimum level substrate temperature of about 500°F.

In the following Table, the result of variations in bias voltage on both the power input density, and the substrate temperature may be seen. The examples were obtained in a set-up identical to that of the previous Table holding a constant system pressure of 50 microns and varying the bias voltage in increments of 500 volts. As may be seen, corresponding increases occurred in current amperage, power input and substrate temperature. It may also be seen that in example 11, the power

55 60 What is claimed is:

1. A method of physical vapor deposition for depositing material on a substrate, comprising, placing a source of evaporant material and a substrate in a vacuum chamber, maintaining an ambient pressure in the vacuum chamber of less than  $10^{-4}$  Torr, heating the evaporant material by means of an electron beam to produce a vapor for deposition on the substrate and intercepting the vapor with the beam of electrons to produce positive ions, and applying an electrical potential to the substrate sufficient to cause ion bombardment of the substrate at a power density of at least about 6 watts per square inch of exposed substrate surface and maintain the substrate at an equilibrium temperature which is at least 25% of the absolute melting temperature of the evaporant.

2. A method according to claim 1 wherein the electrical potential maintained on the substrate is negative d-c with respect to the source.

3. A method according to claim 1 wherein the electrical potential maintained on the substrate is a-c with respect to the source.

4. A method according to claim 1 including the additional steps of sensing the temperature of the substrate and regulating the electrical potential maintained thereon in accordance with the sensed temperature.

\* \* \* \* \*

10

15

20

25

30

35

40

45

50

55

60

65